

Dec. 30, 1947.

W. C. BROWN

2,433,339

APPARATUS FOR BRAZING RADIALLY EXTENDING  
PLATES TO THE INTERIOR OF A TUBE

Filed Feb. 10, 1944



INVENTOR.  
WILLIAM C. BROWN,  
By Elmer J. Gorn  
ATTY.

## UNITED STATES PATENT OFFICE

2,433,339

## APPARATUS FOR BRAZING RADIALLY EXTENDING PLATES TO THE INTERIOR OF A TUBE

William C. Brown, Watertown, Mass., assignor to Raytheon Manufacturing Company, Newton, Mass., a corporation of Delaware

Application February 10, 1944, Serial No. 522,194

6 Claims. (Cl. 113—99)

1

This invention relates to an apparatus for making a multiplex anode structure for a hyper-frequency oscillator tube of the magnetron type. Tubes of the above type have heretofore been made in which the anode structure comprises a plurality of substantially radially disposed anode arms secured to the inner face of a cylindrical anode block. The space between each pair of anode arms constitutes a cavity resonator. Due to the fact that the frequency of the oscillations produced by such a device depends upon the geometrical configuration of such resonators, and since the efficiency of such a device depends in large part upon the accurate matching of the cavity resonators, it is particularly important that the anode plates be accurately secured in place. Heretofore difficulties have been encountered in constructing anodes of the above type and the art has resorted to relatively complex and expensive arrangements for insuring proper construction thereof.

An object of this invention is to devise an apparatus for soldering a plurality of anode arms in place in an anode structure of the above described type in a simple and reliable manner.

Another object is to increase the accuracy with which a tube of the above type may be constructed so as to increase the efficiency of operation thereof as a generator of hyper-frequency oscillations.

The foregoing and other objects of this invention will be best understood from the following description of an exemplification thereof, reference being had to the accompanying drawing wherein:

Fig. 1 is an exploded perspective view partly broken away of the novel apparatus of this invention;

Fig. 2 is a vertical section through the apparatus of Fig. 1 showing the wedge members in their assembled position; and

Fig. 3 is a cross-section taken along line 3—3 of Fig. 2.

The multiplex anode structure which is to be constructed in accordance with this invention comprises a cylindrical anode block 1 made of some suitable highly conductive metal, such as copper, within which are mounted a plurality of anode plates 2 soldered to the inner surface of an annular projection 3 formed upon the inner wall of the block 1. The inner edges of the anode plates 2 form a plurality of anode faces adapted to cooperate with a thermionic cathode (not shown) supported centrally of said anode faces. The space between each pair of anode

arms 2 constitutes a cavity resonator, the geometrical configuration of which determines the frequency of the oscillations to be generated by the completed device. As already pointed out, 5 it is necessary that these cavity resonators be accurately formed. Also it is necessary that a good electrical contact be created between each of the anode arms 2 and the anode block 1. The anode arms 2 are likewise formed of a highly 10 conductive material, such as copper.

In order to construct the anode arrangement as described above, there is provided a jig 4 formed preferably of stainless steel. The jig 4 is provided with a base portion 5 from which 15 projects a central hollow cylindrical portion 6. The anode block 1 is adapted to be placed over the cylindrical portion 6, the lower end of said anode block 1 resting on the base portion 5. The cylindrical portion 6 is preferably of such a 20 height that when the anode block 1 rests on the base portion 5, the upper edge of the annular projection 3 extends slightly above the upper end of the cylindrical portion 6. The cylindrical portion 6 is also provided with a plurality of 25 radial slots 7 extending from the upper end of said member 6 to substantially the lower end of the annular projection 3. The formation of the slots 7 in the member 6 leaves a plurality of intervening arm members 8. The outside diameter of the cylindrical member 6 is somewhat less 30 than the inner diameter of the annular projection 3. Each of the arms 8 is provided with a pair of projections 9 extending outwardly for a sufficient distance so as to contact the wall 35 of the annular projection 3. The projections 9 are each tapered so as to provide only a limited area for thus contacting the wall of said projection 3.

After the anode block 1 is placed on the jig 4, 40 a plurality of plates forming the anode arms 2 are inserted in the slots 7. These plates 2, when resting upon the bottoms of the slots 7, will thus be supported at the proper level with respect to the annular projection 3. In order to force 45 the anode arms 2 into an intimate contact with the wall of the annular projection 3, and in order to hold the anode plates accurately and firmly in this position, there is provided a lower wedge member 10 and an upper wedge member 11. The lower wedge member 10 is provided with a tapered surface 12, the upper end of which is somewhat smaller than the desired final diametric 50 distance between oppositely disposed anode arms 2, and the lower end of which is slightly greater than this distance. The upper wedge member

11 has a tapered surface 13, the lower end of which is slightly smaller than the above defined final diametric distance between oppositely disposed anode arms 2, and the upper end of which is slightly larger than said distance. The lower wedge member 10 is provided with a projecting rod 14 which is adapted to fit into a central opening 15 provided in the upper wedge member 11 so as to guide said wedge members into alignment.

After the anode plates have been assembled as described above, the wedge members 10 and 11 are inserted into the structure, as shown in Fig. 2, and said wedge members are forced toward each other. The tapered surfaces 12 and 13 engage the lower and upper portions respectively of the outer edges of the anode plates 2 and force said anode plates into intimate engagement with the inner wall of the annular projection 3. The wedge members are likewise preferably formed of stainless steel.

In order to solder the plates 2 in position, a solder ring 16 is laid upon the top surface of the anode plates 2 immediately adjacent the annular projection 3. The solder ring is preferably made of eutectic alloy of copper and silver. The solder ring 16 is formed so as to possess a certain degree of resilience. The plates 2 are slightly shorter than the annular projection 3 which thus permits the solder ring 16 to be sprung into position engaging the exposed upper portion of the annular projection 3.

After the parts have been assembled as described above, the assembly is placed in a furnace which preferably has a predominantly hydrogen atmosphere. The furnace raises the temperature of the assembly to a point at which the solder 16 melts. It has been found that when such melting occurs the solder runs down along the inner wall of the projection 3 and penetrates into the region between each anode plate 2 and said annular projection. In this way, each of the anode arms 2 is securely soldered in place. It has been found that the soldered joints thus produced are very strong mechanically and have a very high electrical conductivity.

The jig 4 and the wedge members 10 and 11 being made of stainless steel have little if any tendency to stick to the solder. To this extent such stainless steel members may be said to be solder repellent. Moreover it will be noted that the members 10 and 11 nowhere come into contact with the solder 16 and the only places where the member 4 comes into contact with such solder are at the outer ends of the projection 3. As already pointed out, these are of limited area so that if any tendency to stick exist at these points, the areas are sufficiently restricted so that the jig 4 may be readily pulled away from the anode structure after the soldering has been completed.

It has been found that anodes may be constructed in accordance with the foregoing with a high degree of accuracy and with great ease and facility.

Of course it is to be understood that this invention is not limited to the particular details as described above, inasmuch as many equivalents will suggest themselves to those skilled in the art. It is accordingly desired that the appended claims be given a broad interpretation commensurate with the scope of the invention within the art.

What is claimed is:

1. Apparatus for use in soldering, comprising: a cylindrical jig member having a longitudinally extending opening, a plurality of substantially

radially extending slots passing through the wall of said jig member, said slots extending from one end of said jig member to a distance short of the other end of said jig member, and a pair of wedge members of circular cross-section adapted to be inserted respectively into the upper and lower ends of said longitudinally extending opening, the cross-section of each of said wedge members varying between greater and less than the diameter of said longitudinally extending opening.

2. Apparatus for use in soldering, comprising: a cylindrical jig member having a longitudinally extending opening, a plurality of substantially radially extending slots passing through the wall of said jig member, said slots extending from one end of said jig member to a distance short of the other end of said jig member, a plurality of projections on the outer wall of said jig member, said projections having their outer ends of limited area lying in a cylindrical surface of diameter substantially greater than the outer diameter of the wall of said jig member, and a pair of wedge members of circular cross-section adapted to be inserted respectively into the upper and lower ends of said longitudinally extending opening, the cross-section of each of said wedge members varying between greater and less than the diameter of said longitudinally extending opening.

3. Apparatus for use in soldering, comprising: a cylindrical jig member having a longitudinally extending opening, a base portion, and an upper cylindrical portion of a diameter substantially less than said base portion, a plurality of substantially radially extending slots passing through the wall of said jig member, said slots extending from one end of said jig member to a distance short of the other end of said jig member, and a pair of wedge members of circular cross-section adapted to be inserted respectively into the upper and lower ends of said longitudinally extending opening, the cross-section of each of said wedge members varying between greater and less than the diameter of said longitudinally extending opening.

4. Apparatus for use in soldering, comprising: a cylindrical jig member having a longitudinally extending opening, a plurality of substantially radially extending slots passing through the wall of said jig member, said slots extending from one end of said jig member to a distance short of the other end of said jig member, a pair of wedge members of circular cross-section adapted to be inserted respectively into the upper and lower ends of said longitudinally extending opening, the cross-section of each of said wedge members varying between greater and less than the diameter of said longitudinally extending opening, and a rod extension at one end of one of said wedge members, the other of said wedge members having an opening adapted to receive said rod projection to hold said wedge members in alignment.

5. Apparatus for use in soldering, comprising: a cylindrical jig member having a longitudinally extending opening, said jig member being adapted to support a hollow, cylindrical workpiece about the same, a plurality of substantially radially extending slots in the wall of said jig member, said slots extending from one end of said jig member to a distance short of the other end of said jig member and being adapted respectively to receive a plurality of workpieces to be soldered to said first-mentioned workpiece, and a pair of wedge members within said jig member, engaging the opposite ends respectively of said plurality of workpieces, and holding the same in contact

with the inner wall of said first-mentioned work-piece.

6. Apparatus for use in soldering, comprising: a cylindrical jig member having a longitudinally extending opening, said jig member being adapted to support a hollow cylindrical workpiece about the same, a plurality of substantially radially extending slots in the wall of said jig member, said slots extending from one end of said jig member to a distance short of the other end of said jig member and being adapted respectively to receive a plurality of workpieces to be soldered to said first-mentioned workpiece, a pair of wedge members within said jig member, engaging the opposite ends respectively of said plurality of workpieces, and holding the same in contact with the inner wall of said first-mentioned workpiece, and a body of solder supported in said first-mentioned workpiece, adjacent the points at which said plurality of workpieces contact said first-mentioned workpiece. 15 10 20

WILLIAM C. BROWN.

#### REFERENCES CITED

The following references are of record in the file of this patent:

#### UNITED STATES PATENTS

| Number    | Name    | Date           |
|-----------|---------|----------------|
| 1,541,058 | Lee     | June 9, 1925   |
| 2,186,641 | Jones   | Jan. 9, 1940   |
| 2,310,841 | Curtis  | Feb. 9, 1943   |
| 2,306,291 | Alons   | Dec. 22, 1942  |
| 2,257,643 | Paschke | Sept. 30, 1941 |

#### OTHER REFERENCES

"A Skin Game in Metallurgy," Scientific American, June 1941, pages 331-332, published by Munn and Co., New York.

"Welding Procedures," published by Air Reduction, New York, page 21.